

July 29, 1947.

H. G. SCULL

2,424,857

PROCESS FOR DYEING TEXTILE MATERIALS COMPRISING A  
CELLULOSE CARBOXYLIC ESTER WITH VAT DYES

Filed Oct. 21, 1943



## UNITED STATES PATENT OFFICE

2,424,857

## PROCESS FOR DYEING TEXTILE MATERIALS COMPRISING A CELLULOSE CARBOXYLIC ESTER WITH VAT DYES

Herbert G. Scull, New York, N. Y., assignor to Eastman Kodak Company, Rochester, N. Y., a corporation of New Jersey

Application October 21, 1943, Serial No. 507,144

2 Claims. (Cl. 8—36)

1

This invention relates to a process for dyeing textile materials, such as filaments, threads, yarns or fabrics (knitted or woven) comprising a cellulose carboxylic ester and particularly to a process for dyeing such textile materials with vat dyes.

The dyeing of textile materials, such as cotton and regenerated cellulose rayon, with vat dyes is very well known. The vat dyes can be applied to the textile materials by immersing the materials in a vat containing an alkaline solution of the vat dye in its reduced form, followed by oxidation of the dye on the textile; this is practical in a continuous or stepwise process. Textile materials, such as cotton and regenerated cellulose rayon, can also be dyed with vat dyes by padding the materials with a vat dye in its unreduced form and then subjecting the padded material to the action of an alkaline reducing agent, followed by oxidation. These methods of applying vat dyes to textile materials comprising a cellulose carboxylic ester, however, have not been satisfactory, owing to the fact that the alkaline baths (vats) cause excessive saponification of the cellulose ester material, thereby detrimentally altering its characteristics.

Because some vat dyes are exceedingly stable to light, a number of efforts to devise methods for dyeing textile materials comprising a cellulose carboxylic ester with vat dyes have been made. Some of these have been almost entirely unsuccessful. In other cases, it has been proved possible to apply certain vat dyes to textile materials comprising a cellulose carboxylic ester, but the vat dyes which have been successfully applied are of the simpler types and not stable to light. With the more complex vat dyes such as the anthraquinone vat dyes, many of which are very stable to light and require alkaline reducing agents to effect their reduction, efforts to dye textile materials comprising a cellulose carboxylic ester have not met with success.

Among the earliest proposals for the dyeing of textile materials comprising a cellulose carboxylic ester was that of merely treating the textile material with an aqueous suspension of the vat dye having in its chemical constitution an active group (hydroxyl, amino, nitro, nitroso, etc.) content preponderant numerically over any sulfo group content. This proposal, while possibly suitable for certain low molecular weight dyes, is of no use, whatsoever, in the case of the complex anthraquinone vat dyes. Moreover, such a method would leave cotton and viscose rayon white in fabrics involving a mixture of cellulose carboxylic ester rayon and cotton or viscose rayon. Another

2

early proposal was to treat the textile materials with vat dyes in a vat of such low alkalinity that the cellulose ester was not saponified, the vat containing a protective colloid such as gelatin or starch and a water-soluble salt, such as calcium chloride or sodium chloride. Likewise, this proposal, while possibly suitable for vat dyes of a simple character, is of no utility whatsoever for the high molecular weight complex anthraquinone vat dyes. Still another proposal was to treat the cellulose ester textile material with a vat dye in a vat in which the strong alkali usually employed was replaced with an alkali phenate. This proposal was made largely in connection with efforts to dye mixed textile materials containing both cellulose ester yarn and regenerated cellulose yarn or cotton yarn. However, in operating according to this proposal, it is found that the vat dyes do not color the cellulose ester yarn to deep, full shades so that it is necessary to supplement the vat dyeing with a direct dye for the cellulose ester yarn in order to bring the cellulose ester yarn to the same depth of color as the regenerated cellulose rayon yarn or cotton yarn. Moreover, operating according to this method with light-fast anthraquinone dyes, the dyes obtained on the cotton or the regenerated cellulose rayon are poor "money value" dyeings. Still another proposal has been to color cellulose ester textile materials with ester salts of vat dyes. However, unless special methods of handling are employed, cellulose carboxylic ester rayon cannot be dyed with these dyes and, in any event, only a limited range of colors which are fast to light on cellulose carboxylic ester rayon are available.

I have now found a process for dyeing textile materials comprising a cellulose carboxylic ester with vat dyes, including the light-stable, high molecular weight complex anthraquinone vat dyes. My new process is especially useful in the dyeing of piece goods containing both cellulose carboxylic ester rayon yarn and cotton yarn or regenerated cellulose rayon yarn.

It is, accordingly, an object of my invention to provide a process for dyeing textile materials comprising a cellulose carboxylic ester with vat dyes. Other objects will become apparent hereinafter.

In accordance with my invention, textile materials comprising a cellulose carboxylic ester, in which the acid radical contains from 2 to 4 carbon atoms, are padded with a liquid padding mixture comprising a vat dye, such as an anthraquinone vat dye, substantially in its unreduced form, a stable alkaline reducing agent (i. e., a

reducing agent which is substantially inactive below 140° F. in alkaline medium) for the vat dye, an alkaline agent and a thickening agent. The dye-padded textile material is then advantageously dried without contact of its useful surface with any object during the initial part of the drying operation in which sufficient volatile liquid is removed from the padded textile material so that smearing will not occur upon contact of the textile material with any object. Promptly following drying, the textile material is aged, i. e., treated with steam until the vat dye is substantially reduced and the cellulose carboxylic ester fibers are saponified to a greater or lesser degree on their surfaces. The saponification obtained in this manner is not to be confused with the saponification which occurs in an alkaline vat. The saponification which obtains in practicing my invention is a surface saponification which, I have found, is essential in order to obtain dyeings with anthraquinone vat dyes. Following aging, the textile material is treated with an oxidizing agent for the reduced vat dye in order to convert the dye to the unreduced or oxidized form. Following development of the color by oxidation, the textile material is washed with water and dried.

My invention is not to be confused with the prior-printing processes wherein vat dye pastes are printed upon textile materials in various designs, the materials dried, aged and developed. In these prior-printing processes, the textile material is printed on one side only at one time, and piece goods travel but a relatively short distance from the printing roller before the goods are supported by some means such as rollers during the drying process. While such a method of drying can be employed in printing processes, such methods cannot be employed in my new process where the textile material is padded throughout its thickness with the padding mixture, since the solid support, such as the roller, would cause smearing on the dyed surface of the material. With cotton or regenerated cellulose rayon textile materials, no problem of support during drying arises, since even the unreduced dyes are much more readily taken up by these textile materials than is the case with cellulose ester materials, and the cotton fibers or regenerated cellulose fibers, therefore, may be supported on rolls or the like with the entire surface (or width) of the fabric resting upon the support while the fabric is still wet with the padding solution. On the other hand, any attempt to support by means of smooth rollers a textile material comprising cellulose carboxylic ester fibers, while still wet with the padding mixture, would result in smearing of the dye which is only on the surface of each carboxylic ester fiber at that point in the process. Moreover, in printing processes the textile material is pulled under considerable tension in order to obtain proper registration of the pattern. Contrasted with printing processes, the textile material in my new process is under substantially no tension, i. e. it is not pulled excessively during or after padding: only sufficient tension is applied to the goods to carry it through the various operations.

This distinction is further emphasized by the fact that printing processes always employ a paste, i. e. a mixture of the various components necessary for printing which mixture has a texture with sufficient body that it is held uniformly in the engravings of the printing rolls until deposited upon the textile material which deposit-

ing occurs uniformly and with a permanent sharp contour for the design being printed; in block screen printing, pastes must be of a sufficient thickness to prevent "flooding" or flowing in the design when the squeegee is moved across the screen. Distinguished from such pastes my process employs a padding mixture in the form of a liquid which readily flows upon the textile material, permeates the fabric and coats the individual fibers of the material. Printing pastes are wholly unsuited for use in my process because they would not spread and permeate the fabric and conversely my liquid padding mixtures are wholly unsuited for printing because they would not be held uniformly in the engraving and would spread over and permeate the fabric.

In practicing my new process, the dye-padded textile material is dried without contact of its useful surface with any object during the initial part of the drying operation. The useful surface of a fabric may be defined as that which is co-extensive with that portion of the fabric normally intended to be made into garments, such as that between the selvages or that between the edge portions that would normally be trimmed off and discarded. When I specify drying of the textile material without contact, I mean without contact during the drying operation. When the padded material leaves the padding rolls it may be batched by rolling the fabric in large rolls but the drying operation should normally follow before atmospheric drying of the exposed edges of the rolled fabric occurs sufficiently to cause migration of the dye. Also the padded fabric may be conducted directly from the padding rolls over an endless blanket or even over smooth rolls so long as such blanket or such rolls are kept clean (in their rotation) and padding mixture is not allowed to accumulate on the surface thereof. I do not regard this portion of the transit of the fabric through my process as being part of the drying operation, as any drying at this point is merely incidental. This drying operation without contact can be accomplished by taking the end of the textile material as it comes from the padding operation and carrying it through a drying atmosphere until the material is dry enough so that it can be passed over a roller or other suitable supporting means without marring the padded surface. Still another method of conducting the drying of the dye-padded material is to support the material in a horizontal position by means of an air cushion. Such a cushion is provided by a suitable blast of air from below and from above the material, the two blasts of air serving to counter-act one another and cushion or support the dye-padded material while it is being passed through the drying atmosphere. Normally I have found that if roughly 40 per cent of the volatile material contained in the padding mixture picked up by the fabric in the padding operation, is removed in the drying operation without contact of the fabric with any object, the fabric may then contact rolls, conveyors or the like without marring the fabric surface.

One manner of practicing my invention is illustrated in the accompanying drawing which is a diagrammatic representation, in section, of one embodiment of my invention. In this drawing, a fabric comprising cellulose carboxylic ester rayon yarn is carried over guide rollers 10 into the box 11 of a padding machine, where, supported by a series of rollers 12, it is thoroughly treated with a padding mixture comprising a

light-fast unreduced anthraquinone vat dye, a reducing agent for the vat dye and an alkaline agent, as hereinafter described. Normally the padding mixture is maintained at room temperature (60° to 80° F.) although I may maintain the mixture at higher temperatures, such as 100° F. or even 150° F. or somewhat more, depending upon whether undue saponification takes place, in which event a lower temperature would be employed. From the box 11, the fabric is carried through padding rollers 13 where it is squeezed, the pressure on the padding rollers being adjusted by means of an adjustment mechanism 14 to leave about 65 per cent, based upon the weight of the fabric, of padding mixture in the fabric. From the padding rollers 13, the fabric is taken by its end, carried over fabric covered roller 15 (constructed with an endless belt of blotting cloth as described in Bromley U. S. Patent No. 2,175,051, dated October 3, 1939) and then carried into a drying tower through an opening in the bottom of the left-hand casing 16. Air, which may be preheated, is blown into the tower on either side of the fabric through inlets 17 and is directed upwards in the tower by means of baffles 18. Heating elements, such as steam coils 19, are positioned on either side of the casing 16. The fabric is carried to a height which permits the fabric to become dry enough that contact with a solid object will not mar or smear the padding mixture on the fabric. This height, of course, will vary depending upon the efficiency of the drying atmosphere in the drying tower and the rate at which the fabric is moved through the drying tower. The rate at which the fabric moves through the drying tower is determined by the weight of the fabric and may vary from a few yards per minute for heavy constructions to 125 yards or even more per minute for very light materials, for example. When the fabric is dry enough to be brought in contact with an object, it is carried over a guide roller 20 and downwards through the right-hand casing 21 which contains outlets 20 for air, and thence out of the drying tower. The fabric is then carried across guide rollers 23 and 24 and into a steam chamber wherein it returns over a guide roller 25. In this steam chamber, the fabric is subjected to an atmosphere of moist steam above 212° F., admitted to the steam chamber through perforated steam pipes 26 which are positioned in water wells 27. The steam chamber contains heating elements, such as steam coils 28 positioned on its walls. The steam coils aid in preventing condensation of the steam which travels upwards in the chamber and escapes through a valve 29 which can be adjusted to regulate the flow of steam. Condensation of the steam near the top of the chamber is also retarded by a steam chest 30 which is equipped with a drain 31. In the steam chamber the surface of the cellulose carboxylic ester rayon yarn is saponified and the anthraquinone vat dye is reduced. From the steam chamber, the fabric issues across guide rollers 32 and 33 into an oxidizing bath contained in a tank 34. In the oxidizing bath the fabric is thoroughly treated with an oxidizing mixture (as described hereinafter) while supported on rollers 35, followed by a skying operation, if necessary, in order to oxidize the reduced anthraquinone vat dyes. From the oxidizing bath, the fabric issues over a guide roller 36 and is carried to skying, washing and drying operations.

My invention is directed to the dyeing of textiles containing any percentage (from 1 to 100%)

of cellulose carboxylic ester rayon fibers, filaments or yarn, with any kind of vat dye especially light-fast anthraquinone vat dyes. Moreover, my invention is further especially directed to the dyeing of textiles containing both regenerated cellulose yarn (e. g., viscose yarn or cuprammonium yarn), cotton yarn or wool yarn and cellulose carboxylic ester yarn, with light-fast vat dyes, which dye both yarns to the same cast and approximately the same depth. Vat dyes which are affected by atmospheric acids should be avoided. The following vat dyes have been found to be unaffected by atmospheric deterioration and fast to light for at least 40 hours in light shades when applied to cellulose acetate yarn:

- 20 Dyes listed under Color Index No. 1151, e. g., Indanthrene Brown RAP (paste)  
 20 Dyes listed under Color Index No. 1097, e. g., Carbanthene Golden Orange RRT (paste)  
 Dyes listed under Color Index No. 1152, e. g., Calcosol Brown G Dbl. Pst.  
 Dyes listed under Color Index No. 1150, e. g., Ponsol Olive AR Dbl. Pst.  
 25 Dyes listed under Color Index No. 1173, e. g., Cibalone Blue 3G Dbl. Pst.  
 Dyes listed under Color Index No. 1162, e. g., Calcosol Red BN Dbl. Pst.  
 30 Dyes listed under Color Index No. 1096, e. g., Indanthrene Golden Orange GA Pst.  
 Dyes listed under Color Index No. 1101, e. g., Ponsol Jade Green Dbl. Pst.  
 Dyes listed under Color Index No. 1104, e. g., 35 Amanthrene Brilliant Violet RR Pst.

The padding mixture is advantageously prepared by adding a vat dye, such as one of the above vat colors, to water and stock mixture. 40 The stock mixture is advantageously prepared to contain, in addition to the alkaline reducing agent, an alkaline agent and a suitable thickening agent, an antioxidant, a penetrating agent and a dispersing agent. Alkali metal carbonates are advantageously employed as the alkaline agent, although other substances which provide the necessary alkalinity for the reduction of the vat dye and for the surface saponification of the cellulose ester can be employed, e. g., alkali metal hydroxides, mixtures of alkali metal hydroxides and alkali metal carbonates or mixtures of tri-alkali metal phosphates and alkali metal carbonates. Any alkaline vat dye reducing agent can be employed which will not cause substantial reduction of the vat dye in the padding mixture at 80° F. over a period of 24 hours, e. g., sodium formaldehyde sulfoxylate or some other alkali metal aldehyde sulfoxylate, or a metal aldehyde sulfoxylate, such as normal zinc formaldehyde sulfoxylate. As the thickening agent, British gum, starch, vegetable mucilage, dry gum or Supertex gum T-125 (karaya gum) can be used. As antioxidants, phenols, such as hydroquinone or salicylic acid, may be used. Also glucose or alkali metal hydrogen sulfites may be used as antioxidants. As penetrating agents or assistants, glycerines or glycols are advantageously employed. Diethylene glycol is an especially useful assistant. As dispersing agents, Tergitol 70, Nov. 4 (sodium sulfate of higher secondary alcohols), sulfite cellulose waste liquors, butylated naphthalene sulfonic acids or dipotassium glycol disulfate can be used.

The following example will serve to illustrate further the manner of practicing my invention:

## Example

A stock mixture was prepared by making a solution of the following materials:

|                                 |    |     |
|---------------------------------|----|-----|
| Sodium carbonate                | oz | 16  |
| Formaldehyde sodium sulfoxylate | oz | 27  |
| Hydroquinone                    | oz | 3   |
| Water                           | qt | 2.5 |

and adding thereto the following substances:

|                                                                                       |    |      |
|---------------------------------------------------------------------------------------|----|------|
| Supertex gum T-125 (Jacques Wolf & Co., Passaic, New Jersey) (solubilized karaya gum) | qt | 1    |
| Urea                                                                                  | oz | 20   |
| Diethylene glycol                                                                     | oz | 4    |
| Tergitol No. 4 (Carbide & Carbon Chemicals Corporation)                               | oz | 0.25 |

Ten parts by weight of an anthraquinone vat dye, such as Ponsol Olive G Paste was diluted with 10 parts of water, which mixture was then added to 80 parts of the above-described stock mixture to make 100 parts of padding mixture. The resulting padding mixture was placed in a suitable padding machine, such as the padding machine depicted diagrammatically in the accompanying drawing. Piece goods consisting of viscose rayon yarn and 30 per cent cellulose acetate rayon yarn was run through the padding mixture and through the padding rolls, the pressure on the rolls being adjusted to leave about 65 parts of padding mixture in 100 parts of the goods; this is known in the trade as 65 per cent "pick up." As the goods came from the padding operation, it was taken by its end and carried into a drying tower, such as the drying tower depicted diagrammatically in the accompanying drawing, and dried without contact during drying of its useful surface with any object until it was dry enough that contact with a roller did not cause smearing or marring of the dyed surface of the goods. The goods was then passed over a roller and carried out of the drying tower, with only sufficient tension applied to the goods to carry it through the various operations. (The goods should not be pulled excessively during or after padding. Various of the rolls over which the goods passes may be synchronously driven to reduce the tension upon the goods during the various stages of the process, if desired.) The drying was conducted to remove at least 75 per cent of the volatile in the goods after padding. (Better results are obtained with the removal of 85 per cent or 90 per cent or even 100 per cent of the volatile. Drying can be facilitated by the passage of warm air in the drying tower. Heat radiators or infrared radiators can be positioned at advantageous places in the drying tower to facilitate drying.)

After drying the goods, it was drawn directly through a steam chamber, such as illustrated diagrammatically in the accompanying drawing. (The goods can be batched before entering the steam chamber, and, if batched, should be cooled while batched. A chimney ager can be employed as the steam chamber.) In the steam chamber, the goods was subjected to the action of moist steam while the chamber was maintained at a temperature of from 212° F. to 270° F., for from 3½ to 4 minutes. During this steam treatment the cellulose carboxylic ester fibers were saponified on their surface and the vat dye was reduced and thereupon penetrated into the saponified surface of the fibers. Such surface saponification most desirably takes place to a depth

which is only a fraction (the outer fraction) of the radius of the fiber (for instance  $\frac{1}{16}$  to  $\frac{1}{8}$  of the radius) and the concentration and character of the various components of the padding mixture and the temperature and time of the various steps is regulated, generally speaking, so that surface saponification of only a small fraction of the depth of the fiber takes place.

After steaming, the goods was subjected to oxidation. (The goods can be batched before subjecting to oxidation.) While there are various known ways of developing anthraquinone vat dyes by oxidation, an oxidizing bath containing 2 g. of sodium dichromate and 5 g. of 30 per cent aqueous acetic acid per liter is suitable. The goods was immersed in such an oxidizing bath at 105° F. until the vat dye was oxidized. After oxidizing, the goods was skyed and run in rope form through cold water and washed at 180° F. on a machine styled after the Rodney Hunt system. The goods was then rinsed well and either extracted or suctioned and then dried. The goods as processed was found to have been dyed a deep, uniform, olive gray color which was highly resistant to light fading, washing, atmospheric gas fading, crocking, etc., and to have maintained the characteristic feel and hand of the original goods. The stock mixture employed in the above example can also be made up in accordance with the following formulas:

I. A solution of the following materials was prepared:

|                                    |    |     |
|------------------------------------|----|-----|
| Potassium hydroxide                | oz | 7.5 |
| Potassium formaldehyde sulfoxylate | oz | 32  |
| Salicylic acid                     | oz | 3   |
| Water                              | qt | 2.5 |

To the resulting solution were added the following substances:

|                                                |    |      |
|------------------------------------------------|----|------|
| British gum (70% converted, 4 lbs. per gallon) | qt | 1    |
| Urea                                           | oz | 20   |
| Thio-di-glycol ether                           | oz | 4    |
| Tergitol #4                                    | oz | 0.25 |

II. A solution of the following materials was prepared:

|                                 |    |     |
|---------------------------------|----|-----|
| Trisodium phosphate             | oz | 12  |
| Sodium carbonate                | oz | 4   |
| Sodium formaldehyde sulfoxylate | oz | 28  |
| Hydroquinone                    | oz | 3   |
| Water                           | qt | 2.5 |

To the resulting solution were added the following substances:

|                      |    |      |
|----------------------|----|------|
| Supertex T-125       | qt | 1    |
| Urea                 | oz | 20   |
| Thio-di-glycol ether | oz | 4    |
| Tergitol #4          | oz | 0.25 |

III. A solution of the following materials was prepared:

|                                 |    |     |
|---------------------------------|----|-----|
| Sodium hydroxide                | oz | 5.5 |
| Sodium formaldehyde sulfoxylate | oz | 28  |
| Hydroquinone                    | oz | 3   |
| Water                           | qt | 2.5 |

To the resulting solution were added the following substances:

|                                                |    |    |
|------------------------------------------------|----|----|
| British gum (70% converted, 4 lbs. per gallon) | qt | 1  |
| Urea                                           | oz | 20 |
| Triethylene glycol                             | oz | 4  |

IV. A solution of the following materials was prepared:

|                                 |    |     |
|---------------------------------|----|-----|
| Sodium carbonate                | oz | 10  |
| Sodium hydroxide                | oz | 2.5 |
| Sodium formaldehyde sulfoxylate | oz | 28  |
| Hydroquinone                    | oz | 3   |
| Water                           | qt | 2.5 |

To the resulting solution were added the following substances:

|                                                |    |      |
|------------------------------------------------|----|------|
| Supertex T-125                                 | qt | 0.5  |
| British gum (70% converted, 4 lbs. per gallon) | qt | 0.5  |
| Urea                                           | oz | 20   |
| Sodium thiocyanate                             | oz | 4    |
| Tergitol #4                                    | oz | 0.25 |

V. A solution of the following materials was prepared:

|                                    |    |     |
|------------------------------------|----|-----|
| Potassium carbonate                | oz | 16  |
| Potassium formaldehyde sulfoxylate | oz | 32  |
| Hydroquinone                       | oz | 3   |
| Water                              | qt | 2.5 |

To the resulting solution were added the following substances:

|                                                                                  |    |      |
|----------------------------------------------------------------------------------|----|------|
| Supertex gum T-125 (Jacques Wolf & Co., Passaic, N. J.) (solubilized karaya gum) | qt | 1    |
| Urea                                                                             | oz | 20   |
| Diethylene glycol                                                                | oz | 4    |
| Tergitol #4                                                                      | oz | 0.25 |

VI. A paste of the following materials was prepared:

|                                      |    |       |
|--------------------------------------|----|-------|
| Normal zinc formaldehyde sulfoxylate | oz | 16    |
| Sodium formaldehyde sulfoxylate      | oz | 8     |
| Thiodiglycol                         | oz | 2     |
| Sodium carbonate                     | oz | 16    |
| Water                                | qt | 2 1/2 |
| Tergitol #4                          | oz | 0.25  |

Disperse the above paste with a suitable grinding or dispersing machine, i. e., ball mill or colloid mill. Add to the dispersed mass: 1 qt. British gum (70% converted, 4 lbs. per gallon).

In a manner similar to that illustrated in the above example, any other textile materials comprising cellulose carboxylic esters can be vat dyed. For instance, one may desire to employ much higher percentages (than referred to in the above example) of cellulose acetate fibers in the fabric to be dyed by my process, e. g., a fabric composed of about equal parts by weight of cellulose acetate rayon and viscose rayon—a fabric not uncommon in the trade, or a fabric constructed of 60 per cent spun cellulose acetate rayon and 40 per cent cellulose acetate filament yarn. Textile materials comprising 100 per cent cellulose carboxylic esters should not be excessively pulled under any circumstances. Again some fabric constructions may employ 50 per cent acetate and approximately 25 per cent viscose and 25 per cent cotton; such fabrics can readily be dyed by my process. Again some fabrics may be predominately viscose or predominately cotton and have reason to contain only a few per cent (such as 20 per cent or 10 per cent) of cellulose carboxylic ester fibers such as cellulose acetate; such fabrics can readily be dyed by my process. In fact, as above stated, my process has application to any fabric containing any percentage from 1 to 100 per cent, by weight, of cellulose carboxylic ester fibers, filaments or yarns. As explained, the viscose or cotton content of the fab-

ric dyes readily and furnishes no particular problem; however, the cellulose carboxylic ester fibers, as pointed out do not readily absorb vat dyes. By utilizing my process, fabrics containing cellulose carboxylic ester fibers or filaments are handled in such a manner that the padding mixture containing the dye is evenly deposited on the surface of the cellulose carboxylic ester fibers and dried before contact of the coated fibers with any object; the drying step acts to cause the padding mixture to cling with sufficient adhesivity to the fiber surface to permit the fabric to be handled without disturbing the coating. The reduction step (steaming) performs a two-fold function in

that the surface of the cellulose carboxylic ester fiber is saponified sufficiently to permit the dye to penetrate the fiber and the dye is at the same time reduced to a form which is readily absorbed by the saponified surface. Thus by a combination of all of these steps, I have been able to obtain even and permanent dyeings of cellulose carboxylic ester fibers, which result has not, to my knowledge, been possible heretofore in the art.

Cellulose carboxylic esters which are employed in the manufacture of textile materials include the partially hydrolyzed as well as the unhydrolyzed cellulose acetates, cellulose propionates, cellulose butyrates and the partially hydrolyzed as well as the unhydrolyzed mixed esters of cellulose, such as cellulose acetate-propionate and cellulose acetate-butyrate. All of these cellulose carboxylic esters consist of a cellulose portion or radical and an acid radical which contains from

2 to 4 carbon atoms and fabrics containing fibers, filaments or yarns of all such esters can readily be dyed by my process. However, when employing textile materials made from yarn which is made from cellulose carboxylic esters containing higher percentages of acid radicals, e. g. the above-mentioned unhydrolyzed cellulose carboxylic esters, the saponification should be effected to a greater extent than when employing textile materials made from yarn which is made from cellulose carboxylic esters containing lower percentages of acid radicals, e. g., partially hydrolyzed cellulose carboxylic esters. Greater saponification can be obtained by extending the time of steaming operation and/or by increasing the concentration of the alkaline agent.

Typical vat dyes are described in "The Synthetic Dyestuffs and Intermediate Products," by Cain and Thorpe, 7th ed (1934), Lippincott Company, Philadelphia, page 226 et seq.

What I claim as my invention and desire to be secured by Letters Patent of the United States is:

1. A process for uniformly dyeing in solid color throughout its thickness a fibrous textile material comprising cellulose carboxylic ester fibers, in which ester the acid radical contains from 2 to 4 carbon atoms, without detrimentally altering the physical characteristics of the original fibers of the textile material, comprising padding the textile material throughout its thickness with a liquid padding mixture comprising a substantially unreduced vat dye, sufficient alkaline reducing agent which is substantially inactive at temperatures up to 140° F. to accomplish reduction of the vat dye, and sufficient alkaline agent to convert the reduced vat dye to its salt form and to cause surface saponification of a small fraction of the depth of the ester fibers, drying the padded textile material at an elevated temperature, while maintaining it in a horizontal position by means of an air cushion, without contact of its useful

surface with any object during the drying operation until the padding mixture on the material is dry enough that it will not smear upon contact with a solid object, steaming the dried textile material at a temperature of from about 212° F. to about 270° F. in order to reduce substantially completely the vat dye and in order to saponify the surface of the cellulose carboxylic ester fibers, and treating the steamed textile material with an oxidizing agent to oxidize the reduced vat dye.

2. A process for uniformly dyeing in solid color throughout its thickness a fibrous textile material comprising cellulose carboxylic ester fibers, in which ester the acid radical contains from 2 to 4 carbon atoms, without detrimentally altering the physical characteristics of the original fibers of the textile material, comprising padding the textile material throughout its thickness with a liquid padding mixture comprising a substantially unreduced anthraquinone vat dye, sufficient alkali metal formaldehyde sulfoxylate reducing agent which is substantially inactive at temperatures up to 140° F. to accomplish reduction of the anthraquinone vat dye, and sufficient alkali metal carbonate to convert the reduced anthraquinone vat dye to its salt form and to cause surface saponification of a small fraction of the depth of the ester fibers, drying the padded textile material at an elevated temperature, while maintaining it in a horizontal position by means of an air cushion, without contact of its useful surface with any object during the drying operation until the padding mixture on the material is dry enough that it will not smear upon contact with a solid object, steaming the dried textile material at a temperature of from about 212° F. to about 270° F. in order to reduce substantially completely the anthraquinone vat dye and in order to saponify the surface of the cellulose carboxylic ester fibers, and treating the steamed textile material with an oxidizing agent to oxidize the reduced anthraquinone vat dye.

3. A process for uniformly dyeing in solid color throughout its thickness a fibrous textile material comprising cellulose acetate fibers, without detrimentally altering the physical characteristics of the original fibers of the textile material, comprising padding the textile material throughout its thickness with a liquid padding mixture comprising a substantially unreduced anthraquinone vat dye, sufficient alkaline reducing agent which is substantially inactive at temperatures up to 140° F. to accomplish reduction of the anthraquinone vat dye, and sufficient alkaline agent to convert the reduced anthraquinone vat dye to its salt form and to cause surface saponification of a small fraction of the depth of the cellulose acetate fibers, drying the padded textile material at an elevated temperature, while maintaining it in a horizontal position by means of an air cushion, without contact of its useful surface with any object during the drying operation until the padding mixture on the textile material is dry enough that it will not smear upon contact with a solid object, steaming the dried textile material at a temperature of from about 212° F. to about 270° F. in order to reduce substantially completely the anthraquinone vat dye and in order to saponify the surface of the cellulose acetate fibers, and treating the steamed textile material with an oxidizing agent to oxidize the reduced anthraquinone vat dye.

4. A process for uniformly dyeing in solid color throughout its thickness a fibrous textile material

comprising cellulose acetate fibers, without detrimentally altering the physical characteristics of the original fibers of the textile material, comprising padding the textile material throughout its thickness with a liquid padding mixture comprising a substantially unreduced anthraquinone vat dye, sufficient alkali metal formaldehyde sulfoxylate reducing agent which is substantially inactive at temperatures up to 140° F. to accomplish reduction of the anthraquinone vat dye, and sufficient alkali metal carbonate to convert the reduced anthraquinone vat dye to its salt form and to cause surface saponification of a small fraction of the depth of the cellulose acetate fibers, drying the padded textile material at an elevated temperature, while maintaining it in a horizontal position by means of an air cushion, without contact of its useful surface with any object during the drying operation until the padding mixture on the textile material is dry enough that it will not smear upon contact with a solid object, steaming the dried textile material at a temperature of from about 212° F. to about 270° F. in order to reduce substantially completely the anthraquinone vat dye and in order to saponify the surface of the cellulose acetate fibers, and treating the steamed textile material with an oxidizing agent to oxidize the reduced anthraquinone vat dye.

5. A process for uniformly dyeing in solid color throughout its thickness a fibrous textile material comprising cellulose acetate fibers, without detrimentally altering the physical characteristics of the original fibers of the textile material, comprising padding the textile material throughout its thickness with a liquid padding mixture comprising a substantially unreduced anthraquinone vat dye, sufficient sodium formaldehyde sulfoxylate reducing agent to accomplish reduction of the anthraquinone vat dye, and sufficient sodium carbonate to convert the reduced anthraquinone vat dye to its salt form and to cause surface saponification of a small fraction of the depth of the cellulose acetate fibers, drying the padded textile material at an elevated temperature, while maintaining it in a horizontal position by means of an air cushion, without contact of its useful surface with any object during the drying operation until the padding mixture on the textile material is dry enough that it will not smear upon contact with a solid object, steaming the dried textile material at a temperature of from about 212° F. to about 270° F. in order to reduce substantially completely the anthraquinone vat dye and in order to saponify the surface of the cellulose acetate fibers, and treating the steamed textile material with an oxidizing agent to oxidize the reduced anthraquinone vat dye.

HERBERT G. SCULL.

#### REFERENCES CITED

The following references are of record in the file of this patent:

#### UNITED STATES PATENTS

| Number    | Name            | Date          |
|-----------|-----------------|---------------|
| 2,205,032 | Chambers et al. | June 18, 1940 |
| 2,067,927 | Kern            | Jan. 19, 1937 |
| 2,107,526 | Dreyfus         | Feb. 8, 1938  |
| 2,318,133 | Wentz           | May 4, 1943   |
| 2,089,920 | Aubauer         | Aug. 10, 1937 |

## 13

| Number    | Name     | Date          |
|-----------|----------|---------------|
| 893,384   | Schlegel | July 14, 1908 |
| 2,080,254 | Dreyfus  | May 11, 1937  |
| 2,164,930 | Lubs     | July 4, 1939  |
| 2,233,101 | Kern     | Feb. 25, 1941 |

## FOREIGN PATENTS

| Number  | Country       | Date          |
|---------|---------------|---------------|
| 376,797 | Great Britain | July 11, 1932 |
| 295,579 | Great Britain | Oct. 17, 1929 |

## 14

## OTHER REFERENCES

Knecht et al., Principles and Practice of Textile Printing, 3d ed., London 1936, pp. 964 and 965.  
 Knecht, Princip. Prac. Textile Printing, 3d ed., London 1936, pg. 3.  
 Hopkins: Journ. Soc. Dyers & Colourists, Dec. 1941, vol. 57, pp. 358-362.  
 Deady: Am. Dyestuff Rep., Nov. 15, 1937, pp. 691-4.  
 Rayon Textile Monthly, Nov. 1944, pp. 82, 85, 86.